

May 26, 1936.

A. W. MORRIS

2,042,409

METHOD OF CASTING METALS

Filed Dec. 22, 1933



INVENTOR

ALBERT WOOD MORRIS  
BY  
Chapin & Neal  
ATTORNEYS

## UNITED STATES PATENT OFFICE

2,042,409

## METHOD OF CASTING METALS

Albert Wood Morris, Springfield, Mass.

Application December 22, 1933, Serial No. 703,568

5 Claims. (Cl. 22—200)

This invention relates to a method of casting metals, particularly such metals as stainless steel, malleable iron, grey iron, and alloy steel, or castings of like metals that must be melted at very high temperatures—say above 2000° F.

The main object of the invention is to improve and maintain a high metallurgical character in the castings and avoid certain defects in castings of such metals as I have found to occur in the methods of casting them as heretofore carried out in practice. Other objects are to make savings in the business of casting such metals apart from and in addition to the superior metallurgical quality.

So far as I am aware, such metals have heretofore been handled as follows: They have been melted within a furnace where the atmosphere in contact with the metal bath has been controlled or is "ideal" for the particular metal, as in an open-hearth, air, or electric furnace. The molten metal has then been "tapped" and taken from the furnace to the molds, and the desired pieces cast by pouring the metal into the molds.

In practice I have found the following objections to this common method. When the metal is taken from the furnace it cools rapidly before being poured for casting. To offset this the metal is superheated, which is costly and bad metallurgically. The pouring temperature for different castings varies widely. The metal is not ordinarily maintained at the best casting temperature for the desired metallurgical results in the casting, and the castings are not uniform. But perhaps more important than the difficulty in the fact that temperatures vary widely between the furnace and the molds, there is the common difficulty of varying atmospheric conditions. When the metal is taken from the furnace in a ladle it is soon exposed to and contaminated by the outside air both before pouring and as the metal is poured into the molds. And the molds are full of gases and air that also contaminate the metal poured into their cavities, as do also the surfaces of the molds. These difficulties have not been entirely overlooked. I am aware that much work has been done to improve the methods of handling hot metals between the furnaces and the molds and to prepare the molds for receiving the metal. But so far as I know, such improved methods are expensive and the results have not yet been satisfactory in metals melting at very high temperatures like steel, for in one way or another such metal is contaminated more or less during the transition time between furnace and mold or in the mold, and such metal is

particularly susceptible to contamination by the exposure to an atmosphere other than one specially prepared for the particular metal.

This is particularly true of metals at very high temperature—2000° F. and above. These metals to which my invention relates commonly need to be poured as the molds are being filled. I am aware of the casting methods in which the molds are filled by suction action or by pressure causing mold filling movement of metal from a suitable reservoir. Without going into the distinctions in detail, one skilled in the art knows that these prior casting methods are not suitable for general application; they are expensive; and they have not and apparently cannot be used in a great many places where the casting molds must be filled by the metal pouring methods as distinguished from suction, pumping, or immersion methods. In many instances the expense is too great. But with metals at temperatures above 2000° F. substantially all casting is done under metal pouring steps to fill the molds. It is in this field that my invention particularly applies for obtaining improved results.

According to the main idea of my invention I can pour the metal in the usual way to fill the mold, but I eliminate the time element in the common practice of transferring the metal from the furnace to position for pouring it into the casting molds. To do this I carry the casting mold to the melting furnace, insert it in the furnace, pour the metal to fill the mold while both mold and metal are in the furnace, and then either remove the mold with its casting from the furnace, or I may remove the casting from the mold while it is still in the furnace. In such operations there is a time element in the step of pouring the metal from the molten mass to fill the mold. But this mold filling step by pouring, takes place while the mold is in the furnace and the operation is possible without using any time during which the molten metal is in transit between the furnace and any point outside of the furnace, and without exposing the metal while being poured to an atmospheric condition different from that in the furnace. The metal is put in the mold before the metal leaves the furnace, and in its cast condition the metal is taken from the furnace either with or without the mold, as I will describe. Thus, there is no chance for contamination of the molten metal by transporting it between the furnace and the mold, and yet the mold is filled by the desired and simple pouring step as from a ladle. Furthermore, by inserting the mold into the

melting furnace long enough for the ladle pouring operation, the interior mold surfaces and the cavities formed by them are prepared in an effective way for taking the hot metal under the best conditions. The extremely high temperature of the furnace will act instantly on said surfaces to dry them. It will also act instantly on all the gases imported in the mold cavities to the furnace and drive them out of the mold by such expansion. So before the mold can be filled these cavity gases (which cause so much trouble in the common casting practices) are driven out and dissipated in the much larger body of gases above the molten mass of metal. Thus the cavity atmosphere before pouring will be substantially the same as the furnace atmosphere above the molten mass. That atmosphere is normally and suitably controlled according to the character of molten metal mass and is one that does not contaminate the metal. It is an entirely different atmosphere than obtains in the mold cavities and against the surfaces of the metal as treated in the common casting practise where the metal is carried from the furnace and poured from a ladle to the mold.

In the accompanying drawing I have shown a cross-section through an open-hearth furnace wherein my method can be carried out.

My method may be carried out in practice by labor-saving apparatus of various kinds coordinated for the purpose, but it may be carried out by hand operations, and I want to emphasize that no expensive apparatus is needed. I herein refer to the hand method tools only, as the features of the new method may best be understood without complicating the description with details of apparatus that would be used to save labor and time. The novel features of my preferred form of apparatus will be the subject matter of additional applications.

Referring to the drawing, I may melt the metal, stainless steel for example, in an open-hearth furnace represented in the drawing at A. The melted metal rests on the hearth B and is at very high temperature when ready for casting, but need not be superheated. A characteristic of stainless steel is that given any opportunity it will absorb carbon with great avidity. It is an alloy and the less carbon it contains the less proportion of expensive elements is necessary in the alloy to give the stainless results. It is also susceptible to contamination in other respects. This is one reason that its castings made in the ordinary way are frequently defective.

I leave the molten body of stainless steel in the furnace and do my casting in the furnace. The open-hearth furnace has a controlled atmosphere of hot gases passing over the surface of the melted bath. They are controlled so that the composition of the alloy will remain as wanted in the casting. Furthermore, these furnace gases maintain the desired temperature in the liquid, such temperature of the metal being easy to control when it is in a large mass and kept in the furnace. I make use of this situation by holding the temperature and atmosphere above the furnace metal at the point best suited to casting. Ordinarily the furnace temperature needs to be kept far above the best casting point so as to compensate for the loss of heat when the metal is transported from the furnace to the molds. And when thus transported the metal is commonly poured in an atmosphere and at a temperature, both outside and inside the mold, that

are not so good as the furnace atmosphere and temperature.

With the temperature in the furnace held as stated, one workman may insert the mold held by a handle, and another the ladle held by a handle, through opposite doors (indicated at C) and made to open and close for my purpose, in the furnace. The workman with the ladle dips metal from the furnace bath (avoiding any slag or dross on the top as is common in ladling hot metal) and pours the metal to fill the mold; or the ladle and mold may be inserted and operated from the same side of the furnace through one door only. The doors being open will not affect the furnace gases to any substantial extent, as the air let in will follow the draft beyond the casting point.

The advantages in filling the mold by pouring the metal under these conditions are that its surfaces and cavities are nicely prepared by the heat of the furnace for receiving the casting, the time for the molten metal to leave its furnace body and get in to the mold is brought to a minimum, the exposure of the metal as it is being poured is in the atmosphere of the furnace gases and at the same temperature, with a minimum risk of contamination. The pouring from ladle to mold can take place without any danger of pouring too much as all excess drops immediately to the furnace bath, so that wastage or expense of remelting is avoided; the mold may be made to take this into account as by having exit passages to cause a mold circulation of hot metal until its cavities are filled solid. But the most important advantage is in the conditions surrounding the pouring operation for the transfer of metal from the body in the furnace to the cavity in the mold without contaminating exposure to atmospheric or body surfaces of the mold, such as occur in the common mold pouring practice.

In using my method for making malleable castings there is the advantage of moving my molds directly from the furnace where they are filled to the annealing furnace in which the mold may be emptied and the casting annealed with a minimum heat loss; and the less handling between the melting furnace and the annealing furnace, the better their metallurgical character can be safeguarded. The method can be used with the air type of furnace as well as the open-hearth, and in the same way.

The operation of my method with regard to the electric furnace is essentially the same as in the case of the open-hearth furnace, with this and possible additional advantage. A well known type of electric furnace is of the rocking type. As the furnace rocks in its normal operation for temperature transfer, the molten mass can be picked up by a pouring lip and the mold filled by the movement of the furnace as a workman holds the mold within the furnace.

The practical use of the method in a large way will involve the use of labor saving apparatus. For example, on opening the doors C of the open-hearth furnace preparatory to casting, a series of successively arranged molds may be inserted and all be in the furnace. The heat there will prepare all the molds for pouring the metal into them. They can be filled with labor saving ladle equipment and removed from the same door they went in or the opposite door. It will be of advantage in some instances to remove the castings while still in the furnace. This can be provided for by a shelf at the side of the hearth where

the casting can be left. And it will be advantageous in some instances to pass the castings as they are removed from the furnace through a furnace door directly into an annealing oven. 5 One of the doors C may be in a passage from the furnace to an annealing oven and opened to admit the casting from the furnace. The workman can shove it in from the opposite side or conveyors may be used. The advantage will be that 10 the casting will not be subjected to contaminating influences.

15 Stainless steel, malleable iron, grey iron, ordinary steel, and such very high melting point metals are to be cast by pouring the metal under this method, and preferably by use of labor saving apparatus which is not shown herein because not necessary to the method invention per se.

I claim:

20 1. The method of casting high melting point metals which consists in continuously operating a furnace to maintain a substantially constant supply of metal at the right casting temperature and then casting in successive cycles by repeatedly inserting a mold in the furnace, pouring 25 the metal into the mold while in the furnace and entirely subjected to furnace heat and atmosphere, and removing the filled mold from the furnace, all without interrupting the furnace operation.

20 2. The method of casting high melting point metals which consists in maintaining metal at the right casting temperature under a controlled atmosphere in the melting chamber of a furnace, and then casting in successive cycles 35 by repeatedly inserting a mold above the molten metal in such chamber and filling the mold by pouring the metal while in said chamber under the atmospheric conditions of the chamber where the metal is maintained for casting, 40 said successive cycles being carried on from the substantially constant metal supply maintained in the furnace.

3. The method of casting high melting point metals which consists in maintaining a large 45 amount of metal in a furnace hot enough to

cast, moving a casting mold of very small capacity compared to the furnace to a position inside the furnace adjacent the metal, and pouring a very small part of the metal from the furnace into the mold to fill it under the same 5 temperature and atmospheric conditions for the pouring operation as for the furnace operation and repeating the casting steps with successive molds while maintaining the same furnace operation on the large amount of metal to have 10 it ready at all times for filling the said small molds as they are successively filled.

4. The method of casting high melting point metals, which consists in melting a large body of metal in a furnace, holding the temperature 15 of the molten metal at substantially the best point for casting purposes, controlling the atmosphere of the furnace in contact with the surface of the metal substantially free of contaminating influence on the metal, intermittently 20 locating a mold in the furnace long enough for its cavity to be filled with the furnace atmosphere, pouring metal from the body in the furnace to fill the mold while in the furnace, and then removing the mold and its casting from 25 the furnace without interrupting the furnace operation on the remaining metal.

5. The method of casting metals from a furnace such as an open-hearth, air, or electric furnace, in which the highest melting temperatures are used, which consists in melting steel, 30 iron, refractory alloys, and such high melting point metals, and raising such metal to approximately the best casting temperature and maintaining it at such point, intermittently inserting 35 a casting mold into the furnace adjacent the level of the molten metal so as to have its cavity atmosphere and surfaces brought to the same temperature as the metal, and then pouring a small part of the metal with a ladle to fill the 40 mold, and removing it, and repeating the casting cycle while maintaining a large body of the metal under the furnace operation while the successive casting cycles are being carried on.

ALBERT WOOD MORRIS. 45